

May 8, 1928.

M. M. MERRITT

1,668,652

APPARATUS FOR AND METHOD OF TANNING HIDES

Filed April 1, 1922

2 Sheets-Sheet 1

*Fig. 1.*



*Fig. 2.*



*Inventor:*  
*Matthew M. Merritt,*  
*by Emery, Booth, Janney & Varney*  
*Attn:*

May 8, 1928.

1,668,652

M. M. MERRITT

APPARATUS FOR AND METHOD OF TANNING HIDES

Filed April 1, 1922

2 Sheets-Sheet 2



Inventor:  
Matthew M. Merritt,  
by Emery, Booth, Janney & Varney.  
Atts.

## UNITED STATES PATENT OFFICE.

MATTHEW M. MERRITT, OF MIDDLETON, MASSACHUSETTS, ASSIGNEE, BY MESNE ASSIGNMENTS, TO UNITED SHOE MACHINERY CORPORATION, OF PATERSON, NEW JERSEY, A CORPORATION OF NEW JERSEY.

## APPARATUS FOR AND METHOD OF TANNING HIDES.

Application filed April 1, 1922. Serial No. 548,861.

This invention relates to the treating of hides and skins by means of liquids or by liquor containing chemical bodies for the purpose of producing either physical or chemical changes, or both, in the skins and hides undergoing treatment.

One of the chief difficulties heretofore encountered in the tanning of skins or hides through the operation of a machine or other apparatus, designed to reduce very considerably the amount of manual labor involved in the handling of the skins or hides and to lessen even more markedly the time consumed in the tanning operations, has resided in the lack of uniformity in the results attained, not only in respect to different skins or hides but in respect to different portions of the same skin or hide. Ordinarily the amount of tanning liquor handled in the apparatus was very large with no adequate provision for securing uniformity in the strength of the liquor with which the skins or hides were treated at any given time while progressively increasing the strength of the liquor to secure the desired results. Under such conditions it not infrequently happened that the skins or hides, or portions thereof, received insufficient amounts of the tanning substances, or the latter failed for various reasons to penetrate to the interior portions of the skin or hide in which case deterioration of the product would be relatively rapid. In short, it has heretofore been difficult to maintain a high standard of excellence and of uniformity in the quality of the product.

One of the objects of the present invention is to provide for a rapid circulation of the treating liquor so that all parts of the skins or hides in the apparatus may be uniformly bathed by the liquor which is itself maintained at uniform strength and temperature throughout the whole body of the liquor due to the very rapidity of its circulation. It is a further object of the invention to provide an improved apparatus by which uniformity in the strength of the treating liquor may be readily obtained and in which the skins or hides may be subjected to uniform treatment by a relatively small body of treating liquor, the strength of

which may be readily changed from time to time according to the judgment of the operator.

According to applicant's method of tanning skins or hides the latter are alternately immersed in the treating liquor and withdrawn therefrom for suspension in the atmosphere of the treating chamber, the hides or skins being immersed in a relatively small body of treating liquor which is caused to flow by the hides or skins in a violently agitated stream to wash deposits of residue from the freshly immersed hides or skins and to maintain uniformity in the strength of the liquor and to cause it to reach all portions of the surfaces of the submerged hides or skins.

The illustrated apparatus and several of its important features, while especially adapted to the tanning of hides or skins, may have other applications and uses, such, for instance, as those which relate to washing, liming, or coloring operations. As shown, the vat in which the drum revolves is relatively small since it is designed to contain only a small body of liquor which is in constant circulation with the liquor in a small tank at a higher level than the vat and connected thereto by a relatively large pipe through which the liquor may flow freely into the vat, thus creating a swiftly flowing stream of treating liquor in the vat. Preferably, and as shown, the tank while relatively small is of a size to contain all of the treating liquor used at any one time in the apparatus so that the liquor while in the tank may receive additions to its strength in treating substances or diluted, as may be desired. In the illustrated construction, the drum which carries the skins or hides alternately into and out of the treating liquor in the vat is provided with an interior drum over which the hides or skins are lapped so that they are maintained in substantially extended condition as they are submerged in the violently agitated treating liquor, and released successively from closely overlapped relation to each other when adjacent to the tanning liquor, whereby all portions of the skins or hides are insured of equal treatment in a treating liquor main-

tained as nearly as possible of uniform strength.

Other features of the invention and other novel combinations of parts will be described in the detailed specification and pointed out in the appended claims.

In the drawings, which show a preferred form of one embodiment of my invention:

10 Figure 1 is a plan view of a preferred form of apparatus for treating leather;

Fig. 2 is a side elevation thereof;

Fig. 3 is a vertical, longitudinal section through the apparatus shown in Fig. 1, being partly in elevation; and

15 Fig. 4 is a diagrammatic view showing a drum provided with an interior drum principally useful for supporting hides of relatively great length considering the diameter of the exterior drum.

20 Referring to the drawings and to the preferred form of my invention selected for illustrative purposes, I have shown an open drum 6 preferably provided with spaced supporting bars to constitute an open head

25 at each end of the drum which is mounted on a shaft 7 with journal bearings 8, 8. The preferred form of drum illustrated is circumferentially provided with dowels 9 with open spaces therebetween. These dowels

30 are removable so that the skins may be folded thereover or otherwise attached thereto prior to the application of the dowels to the drum. The skins may be held in place in any suitable way, but preferably

35 by a strap or belt 10 (Fig. 1) surrounding the drum and bearing against the outer surfaces of the skins when they pass over the dowels.

In Fig. 3 I have shown the skins hung in 40 the drum, but I have purposely omitted many of the skins, as to illustrate them all would render the drawing confused and make less clear the action of the skins as the drum is revolved. Below the center of the

45 drum, enclosing the lower portion thereof, I have provided a tank 11, preferably having its lower wall fitting relatively close to the outer periphery of the drum so that there will be but little of the material treat-

50 ing liquor which is not actively in contact with the drum and that portion of the contents thereof which is submerged. In the preferred form of my invention illustrated, the drum is immersed approximately one-  
55 fourth of its total diameter in the treating liquor, the tank 11 being somewhat higher to prevent spillage.

In Fig. 4, I have shown the drum provided with an inner drum 22 which is im-  
60 portant in treating certain classes of skins or hides, especially hides of considerable length. This may be used not only for thin and medium thickness hides, but also for sole leather, especially when the latter has  
65 been partially tanned. The operation of

the inner drum is to permit the hides to wrap therearound, thereby minimizing that folding or crumpling thereof which is likely to result in a raised grain. While the hides or skins are lapped over each other on the inner drum so that they are maintained in substantially extended condition as they are being immersed in the violently agitated treating liquor, they are released from closely overlapped relation to each other when adjacent to the tanning liquor so that all surfaces of the hides or skins may be reached by the liquor. Where the inner drum is used, the depth of the liquor should be sufficient to cover a portion thereof. The hides are preferably attached by the butts.

70 In connection with the tank 11, I have shown a supply tank 12 adapted to contain a relatively small volume of material treating liquor. The tank 12 is on a higher level than the tank 11, and is connected therewith by a gravity feed pipe 13 through which the liquor flows by gravity from the tank 12 into the tank 11 and also with a return connection 14 in which is interposed circulatory means exemplified by the centrifugal pump 15 for pumping liquor from the tank 11 into the tank 12. Where the open drum in which the skins are hung is adapted to contain about one hundred hides or skins of say fifteen square feet each, I have found that surprising results are attained by circulating the liquor at a rate approximating or exceeding two hundred gallons per minute.

75 It is highly advantageous that heating elements, exemplified by the steam pipes 16, be supplied, preferably in the side tank 12, so

that the liquor may be kept at a uniform temperature. In tanning hides this tem-

perature is preferably about 100 to 110 degrees Fahrenheit. The flow of liquor from the tank 12 to the tank 11 may be regulated by regulating the rate of flow from the tank 11 to the tank 12. This may conveniently

80 be done by providing the valve 17 in the pipe 14 between the centrifugal pump 15 and the tank 11. The pipe 13 is preferably

so much larger than the pipe 14 that the level of the liquor in the two tanks 11 and

85 12 will be generally the same, that in the tank 12 being only sufficiently higher to cause rapid flow of the liquor through the pipe 13 back into the tank 11.

To admit of emptying the tank 11, the connection of the pipe 14 is adjacent the bottom thereof, and a valve 20 is provided in the supply pipe 13.

90 Thus, when the valve 20 is closed and the pump is continued in operation, the tank 11 will be very quickly emptied. The rapid

95 circulation of a relatively small total volume of liquor, as described, results in a surging of the liquor past the materials being treated and, in the tanning of hides, to

100 which my invention is primarily though not exclusively directed, this surging action not

105

110

115

120

125

130

only provides almost absolutely uniform liquor throughout the entire supply thereof in use at any one time, but also speeds up the tanning operation by producing a superior penetration of the liquor into the hides. As the drum is revolved, in the drum shown in Fig. 3, the hides are subjected to a massaging action, falling upon and rubbing against one another. This is disadvantageous in treating many types of hides, and the type of drum provided with the inner drum illustrated in Fig. 4 minimizes this action, greatly improving the leather, especially relatively large hides. For sole leather, I have found that other methods of mounting the hides, as described in my application, Serial No. 588,606 filed Sept. 16, 1922 are preferable. The drum 18 may be revolved or driven in any suitable way, exemplified by the pulley 19 on the shaft 7. The rate of rotation of the drum may be varied somewhat for different classes of work, but I have found that, where an eight foot drum is provided, the revolution thereof at one to two R. P. M. works most satisfactorily.

In the preferred form of my apparatus illustrated, the hides are immersed about one-quarter of the time and are out in the atmosphere about three-quarters of the time, more or less. While in the atmosphere, the hides are wet with the tanning or other liquor used and the tanning operation continues, being in fact accelerated by the action of the air on the hides when wet with the tanning liquor. In this connection, the evaporation of the water content of the tanning liquor while in the air is believed to accelerate the action of the active material in the liquor on the hides. Where the liquor is circulated at a very high rate, each hide as it is withdrawn from the liquor is coated with a film of liquor which is just as fresh as any other liquor in the entire system, this because all the liquor is swirling and therefore that portion of the tanning operation, while the hide is out of the liquor and the water evaporates therefrom, is to a great extent hastened beyond the corresponding action which would take place if the liquor were not in very rapid circulation. The rate of evaporation in a properly designed system is very high, preferably amounting to at least one-twentieth of the entire volume of the liquor each twenty-four hours. This may or may not be compensated for oftener than every twenty-four hours, but I find that in tanning or re-tanning relatively light leathers, such as upper material, the whole operation may be completed in such a short time that it is necessary that the evaporated water be replaced relatively frequently, even continuously, automatically or otherwise. In the case of re-tans the re-tanning operation may be effected in six to twelve hours. It is also desirable that the tanning extracts or other materials be added progressively to increase the barkometer test of the liquor starting with a relatively low barkometer test liquor, say fifteen degrees for upper leather, followed by a very gradual increase and ending with a sudden increase to a liquor of relatively high barkometer test, such, for instance, as forty-five degrees to eighty-five degrees barkometer depending on the hide. The water and chemicals may be added either separately or in combination with each other. It has been found that the addition of any large percentage of water to a tanning fluid at any one time results in an imperfect mixture so that the leather being treated takes up the water and the absorption of the active tanning material is correspondingly retarded. To this end, I prefer that the water be added to the tanning fluid at approximately the same rate that it is evaporated. This may be effected by an ordinary float valve or in any other suitable way.

The swirling stream of tanning fluid, say from two hundred to four hundred gallons per minute in a tank containing say only eighteen inches of liquor at its point of greatest depth and fitting relatively closely to the wheel, results in a forcing of the liquor against the surface of the submerged hides and consequently results in much greater penetration of the pores thereof than where a still liquor is used, or where a relatively sluggish circulation or flow of the liquor is maintained. This, combined with the progressive evaporation of the water from the liquor on the surface of the emerged hides or skins, I believe to result in the strengthening of the liquor on the hides when emerged because of evaporation of the inactive water content thereof.

The use of my improved apparatus and method not only greatly increases the speed of tanning, but very materially improves the quality thereof, other factors such as the tanning solution and the like being constant. This improved quality for any given tanning solution and quality of hide arises somewhat from the fact that the hides are for a shorter time in contact with the water, which, as is well known, exerts a deleterious action on leather, this being particularly true where the water is combined more or less with various foreign chemical elements. The quality is also improved because of the very nature of the action of the active tanning agents on the hide where impacted thereagainst by swirling action of the liquor and by the subsequent action of the film of liquor which is believed to gradually increase in strength and which acts on the hides as the water is evaporated therefrom during the period of emergence.

By circulating the liquor at an extremely rapid rate, I am enabled to maintain a sub-

stantially constant temperature throughout the entire volume thereof. Where the temperature is kept around 110 degrees Fahrenheit, the liquor is of considerably less specific gravity than where colder and is considerably thinner in consistency. The chemical content of the liquor is, however, substantially the same, considered in terms of percentage, at both high and low temperatures, but the liquor is considerably thinner at the higher temperature, resulting in easier penetration of the skin. The relatively uniform temperature of the liquor at say 110 degrees Fahrenheit renders generally uniform, barring great variations in humidity, the evaporation of the water from the hides when suspended in the air, and the residue, after acting strongly on the hide, tends to become gummy, this gummy substance, including both tans and nontans, being again washed from the hide by the swirling action of the bath when the hide is again immersed in the liquor at the bottom of the tank 11, thereby preventing that premature filling which would otherwise retard penetration and tan. During the filling operation, however, the tannage portion of the gummy material tends to fill the hide and the action of the swirling stream is to drive still further into the hide such elements of the relatively heavy liquor as contribute to filling.

It is highly desirable that the operation of the filling of the hide with tanning material be deferred until the hide is tanned all the way through and the washing action of the rapidly swirling fluid, before referred to, to a large extent washes off the thickened tanning material on the hides as they return into the liquor, thus preventing premature filling. The filling is preferably deferred until after the hide is entirely tanned or practically entirely tanned, at which time the filling may be very readily and rapidly effected by an increase in the chemical content of the liquor so as to provide a barometer of say from 25 to 85 degrees at 110 degrees Fahrenheit, depending on the thickness of the leather used. This is a very important factor in improving the quality of the leather, because, if the leather is prematurely filled with thick and viscous tanning material, the tanning of the interior of the hide is only imperfectly effected and is greatly retarded, with attendant stiffening of the grain side of the leather, causing brittleness and causing the leather to crack.

The supply tank 12 is particularly useful in that it permits the thorough admixture of tanning fluid and the introduction of additional water or of chemical bodies, avoiding at the same time both the disadvantages arising from contact of very weak liquor on the hides, with the resultant absorption of water and retardation of the operation, coupled with injurious action on the

hides, and also permits the active chemical agents to be thoroughly mixed, thus avoiding injury to the hides by having overstrong liquor come in contact therewith. The supply tank 12, pursuant to closure of the valve 20, will hold all the liquor exhausted from the tank 11, thus permitting a thorough draining and drying of the hides after the tanning operation is completed. After the liquor is drawn off from the tank 11, the drum may be continuously revolved during the draining and drying operation, so that when the hides are removed they may be relatively dry and clean. This also results in saving a great deal of the liquor, which may be used again.

Before starting the tanning operation, the grain may be struck by immersing the hide in a weak solution of tanning material, preferably while the hide is maintained relatively still, or, if desired, the grain may be struck in the apparatus illustrated by starting with a very weak solution.

While I have shown and described a preferred form of one embodiment of my invention, it will be understood that changes involving omission, substitution, alteration and reversal of parts, and even changes in the mode of operation, may be made without departing from the scope of my invention, which is best defined in the following claims.

Claims:

1. The method of treating a hide or the like with tanning liquor which comprises alternately suspending the hide in the atmosphere while wet with the liquor for such length of time as to permit evaporation of a portion of the water content of the liquor, thereby leaving on the hide a residue richer in tanning agents than the original liquor, and submerging the hide in a body of the liquor to wash off the residue and to wet the hide again with the liquor preparatory to repetition of the suspension in the atmosphere, and violently agitating said treating liquor by causing it to flow continuously past the hide at the rate of over 100 gallons per minute while introducing the treating liquor at a point below the surface of the body of liquor near one end thereof and simultaneously withdrawing the treating liquor at a point near another end of the body of liquor.

2. The method of tanning a hide or the like which comprises suspending the hide from the periphery of a rotatable drum with the hides hanging interiorly of the drum, rotating the drum relatively slowly and passing a violently agitated stream of hide-treating liquor past the bottom of said drum and through the lower portion thereof, whereby alternately to subject said hides to a partial drying in the atmosphere to leave a residue of lessened water content, and to wash off the residue and mix it with

the main body of treating liquor while again wetting the hide with the treating liquor preparatory to emergence thereof as the drum is further rotated.

- 5 3. The method of tanning hides or the like which comprises subjecting them to the action of a rapidly circulated body of tanning liquor of relatively low barkometer test and relatively rapid penetrating capacity until substantially tanned, and then subjecting them for a relatively short time to the action of a rapidly circulated body of tanning liquor of much higher barkometer test and relatively slower penetrating capacity, thereby to avoid premature filling of the hide with resultant retardation of penetration and tanning at the interior of the hide while securing the desired filling of the hide after tanning is substantially or entirely completed.
- 10 4. The method of tanning heavy hides which comprises initially subjecting them while relatively still to the action of a grain-setting liquor and subsequently continuing the tanning operation by repeatedly and alternately subjecting the hides to the action of a rapidly flowing stream of a tanning agent and to the action of the atmosphere.

15 5. Tanning apparatus comprising, in com-

bination, a main tank for containing tanning liquor, a rotatable drum mounted over said main tank and partially submerged in said main tank, an auxiliary tank of a capacity to contain all the liquor while the apparatus is in use, and circulating means 30 for circulating the liquor rapidly through said main tank, the circulating means comprising a pump and a pipe for carrying the liquor from the main tank to the auxiliary tank and a much larger pipe to conduct the 35 liquor in the reverse direction for causing a rapid flow of liquor through the main tank.

6. Tanning apparatus comprising, in combination, a rotatable drum partially submerged in tanning liquor, means for causing 40 a rapidly flowing stream of liquor to pass through the drum, suspension means for hanging hides from the interior periphery of said drum, and supporting means in said drum for supporting the hides in extended 45 overlapped relation as the drum is rotated to prevent undue folding or bending thereof while releasing said hides from closely overlapped relation generally successively adjacent to the tanning liquor.

50 In testimony whereof, I have signed my name to this specification.

MATTHEW M. MERRITT.